

## UNITED STATES PATENT OFFICE

2,300,880

## PRINTING INK

Donald Robert Erickson and Paul J. Thoma,  
Kalamazoo, Mich., assignors to Michigan Re-  
search Laboratories, Inc., Kalamazoo, Mich.

No Drawing. Application June 2, 1941,  
Serial No. 396,288

6 Claims. (CL 260—32)

This invention relates to improvements in printing ink.

This invention relates to printing inks and particularly to such inks in which a binder which is insoluble in water is employed with a solvent which is miscible with water, the binder being soluble in the solvent and a limited quantity of water, but not in the solvent with an unlimited quantity of water, so that the ink may be used in the presence of relatively high humidities without setting up on the press but so that offset may be prevented by treating the printing ink with water to separate the binder and the solvent when more than a limited quantity of water has been added in this way. Such an ink is disclosed and described in our copending application Serial No. 305,640, filed November 22, 1939, for Printing inks.

The objects of this invention are:

First, to provide a new and improved printing ink of the type described.

Second, to provide such a printing ink which has a greater water tolerance than the ink of our aforesaid application.

Third, to provide such an ink which can be made inexpensively and in which the water tolerance may be controlled by the addition of a small quantity of an inexpensive chemical.

Fourth, to provide such an ink in which fatty acids are employed to give the increased water tolerance.

Further objects and advantages pertaining to details will appear from the description to follow.

We have found that the water tolerance of an ink in which the binder is a resin comprising a rosin modified by an alpha beta unsaturated polybasic acid, such as maleic or fumaric, and in which the solvent is a liquid polyglycol such as diethylene glycol, may be increased if small amounts of fatty acids are added to the ink. When these acids are added and are dispersed through the varnish or ink by means of a roller mill, they increase the water tolerance materially and we believe that this is due to a mechanical action because the fatty acids are not soluble in the liquid polyglycol. We believe that the fatty acids serve as a protective coating to slow up the entrance of moisture into the varnish which might cause the ink or varnish to set up on the plates or rollers if an excess of moisture is present in the surrounding air.

We have found that good results can be obtained by using the following fatty acids: Elaeostearic, ricinoleic, capric, oleic, linoic, isolinoic, linolenic, lauric, myristic and erucic.

These acids may be used individually or may be mixed together. We have found that the following commercial products which consist of the combination of acids which are listed with them are satisfactory for our ink:

|                    |                                |
|--------------------|--------------------------------|
| Cocoanut           | Oleic and linoic acids         |
| Helioline          | Oleic and linoic acids         |
| Isoline            | 90% linoic and isolinoic acids |
| 10 Linseed supra   | Linoic and linolenic acids     |
| Linseed fatty acid |                                |
| split #1           | Linoic and linolenic acids     |
| Myristic           | Lauric acid and myristic       |
| Perilla            | Linoic and linolenic acids     |
| 15 Rapeseed        | Erucic and oleic acids         |
| Soy bean           | Oleic and linoic acids         |
| Sunflower          | Linoic and oleic acids         |

We have found that when fatty acids are used 20 in the inks they flow down the tendency of the inks to set up on the press in excessive humidity conditions, but they do not have any appreciable effect in the small percentages used upon the speed of setting the printed film of ink when 25 subjected to steam or water spray or other means of applying water to prevent offset.

We have found that the addition of the fatty acid is effective in inks made with a resin comprising a rosin modified with an alpha beta unsaturated organic polybasic acid such as maleic or fumaric as a binder. The addition of the fatty acid is also effective in inks in which the resin consists of a terpene hydrocarbon of the formula  $C_{10}H_{16}$ , such as alpha terpinene, beta 30 terpinene, pinene, alpha pinene, beta pinene, dipentene, limonene, or terpinolene, modified by maleic acid or the anhydride thereof or some other alpha beta unsaturated organic polybasic acid. We have found that if the binder of the 35 ink consists of a combination of these resins, the addition of the fatty acid is likewise helpful.

Typical examples of our ink are as follows:  
(1) 100 parts by weight of varnish made from 40 50% by weight of a resin comprising a rosin modified with maleic acid or fumaric acid and 50% by weight of diethylene glycol.

45 3 parts of "Isoline" which consists of 90% of linoic and 10% of isolinoic acids.

50 Suitable pigment in amounts varying with the specific pigment and the coloration desired.

(2) 100 parts by weight of varnish made from 55 50% by weight of a resin comprising a terpene hydrocarbon of the formula  $C_{10}H_{16}$  modified with maleic or fumaric acid and 50% by weight of diethylene glycol.

3 parts of "Isoline" which consists of 90% of linoic and 10% of isolinoic acids.

Suitable pigment in amounts varying with the specific pigment and the coloration desired.

(3) 100 parts by weight of a varnish made from 50% of a mixture of resins comprising a rosin modified by maleic or fumaric acid and a terpene hydrocarbon of the formula  $C_{10}H_{16}$  modified by maleic or fumaric acid and 50% diethylene glycol.

3 parts of "Isoline" which consists of 90% linoic and 10% isolinoic acids.

Suitable pigment in amounts varying with the specific pigment and the coloration desired.

The binder of the varnish need not be entirely made up of the above mentioned resins. If 80% by weight of the varnish is made up from the above named resins and diethylene glycol in the percentages specified, 20% by weight may be made up of phenolic resins, gum or wood rosin, 20 alkyd resin, urea or melamine formaldehyde condensation products and zein, or zein modified with an alpha beta unsaturated organic polybasic acid, or an organic hydroxy acid such as malic, lactic, tartaric or citric, or shellac.

The terms and expressions which have been herein employed are used as terms of description and not of limitation, and there is no intention in the use of such terms and expressions of excluding any equivalents of the features shown and described or portions thereof. It is recognized that various modifications are possible within the scope of the invention claimed.

Having thus described our invention, what we claim as new and desire to secure by Letters Patent is:

1. A printing ink comprising 100 parts by weight of varnish comprising 50% by weight of a resin comprising rosin modified by an alpha

beta unsaturated organic polybasic acid and 50% by weight of a polyglycol, 3 parts by weight of a fatty acid having from 16 to 21 carbon atoms in the chain, and a pigment.

2. A printing ink comprising varnish comprising a resin comprising rosin modified by an alpha beta unsaturated polybasic acid and a polyglycol, a relatively small amount of fatty acid having from 16 to 21 carbon atoms in the chain, and a pigment.

3. A printing ink comprising varnish comprising a resin comprising rosin modified by an alpha beta unsaturated organic polybasic acid and a polyglycol, a fatty acid having from 16 to 21 carbon atoms in the chain, and a pigment.

4. A printing ink comprising 100 parts by weight of a varnish comprising 50% by weight of a resin comprising a terpene hydrocarbon of the formula  $C_{10}H_{16}$  modified by an alpha beta unsaturated organic polybasic acid and 50% by weight of a polyglycol, 3 parts by weight of a fatty acid having from 16 to 21 carbon atoms in the chain, and a pigment.

5. A printing ink comprising a varnish comprising a resin comprising a terpene hydrocarbon of the formula  $C_{10}H_{16}$  modified by an alpha beta unsaturated organic polybasic acid and a polyglycol, a fatty acid having from 16 to 21 carbon atoms in the chain, and a pigment.

6. A printing ink comprising a varnish comprising a resin comprising a terpene hydrocarbon of the formula  $C_{10}H_{16}$  modified by an alpha beta unsaturated organic polybasic acid and a polyglycol, a relatively small amount of fatty acid having from 16 to 21 carbon atoms in the chain, and a pigment.

DONALD ROBERT ERICKSON.  
PAUL J. THOMA.